

## UNITED STATES PATENT OFFICE

2,316,041

## PROCESS FOR SIMULATING HAMMERED METAL

Gerald E. Armentrout, Flint, Mich., assignor to  
E. I. du Pont de Nemours & Company, Wil-  
mington, Del., a corporation of Delaware

No Drawing. Application March 12, 1940.  
Serial No. 323,533

2 Claims. (Cl. 117—37)

This invention relates to improvements in the finishing of metal, wood and other surfaces to simulate hammered metal and multi-toned metallic effects.

Heretofore various methods have been known for producing two-toned finishes and some of these methods produce two-toned metallic effects. Practically all of them, however, require the use of two or more paint products and require at least two separate and distinct finishing operations. The methods involving a single finishing operation have the disadvantage of progressively changing in the liquid state, rendering them impractical for continuous application or repair of previous finish in case of damage.

One of the objects of this invention is to produce from a single liquid paint, supplemented with a spatter coat of thinner, a finish having an uneven surface and a multi-toned effect. Another object of this invention is to provide a coating composition which, when applied to a suitable base material, will dry to a protective coating which simulates the appearance of hammered metal. A still further object of this invention is to provide a coating technique which enables the economical production of a hammered metal finish or multi-toned effect. Still another object of this invention is the provision of compositions capable of producing such an improved finish. Other objects will be apparent as the description of the invention proceeds.

These objects are accomplished by incorporating in a thin oleoresinous, resinous or nitrocellulose vehicle as a base material, a flake metallic powder or paste and a granular pigment, and applying the paint or lacquer by spraying, dipping or brushing in such a manner as to first produce a smooth uniform coating, sufficiently heavy to cover the surface, followed, in five to sixty seconds for the nitrocellulose and resinous products, and from four to thirty minutes for the oleoresinous material, with a coat of thinner applied in such a manner as to strike the surface of the paint or lacquer in the form of small droplets instead of by the conventional mist coating methods. These droplets of thinner, upon striking the paint or lacquer, spread out to form spots or small areas having ridges at the edges of the areas with the central portion or crater of these areas having the color of the finely divided metal, while the edges or rim of the crater has the color of the granular pigment or dye used, thus producing a hammered effect. This is directly opposite to prior art wherein the metal migrates to

the rim of the crater with the granular pigment composing the central portion.

Best results have been obtained by first applying two medium wet coats of the metallic paint or lacquer sufficiently heavy to cover uniformly solid in color in each coat, and, before the material has time to set, due to loss of the volatile constituents, applying the droplets of thinner to the surface with a special spatter gun or equipment adjusted for this effect. The hammered effect develops almost immediately at the impact of the thinner.

The compositions which may be used for carrying out this process may vary greatly as to their ingredients and proportions. It has, for example, been found that good results can be obtained by using, as the clear vehicle, either oleoresinous varnishes, alkyd resins of the oil modified type, or clear nitrocellulose lacquers. The vehicles can be chosen so as to be suitable for air drying, for baking or for both.

The base material may be either pigmented or unpigmented, as desired. In order, however, to produce a finish simulating more closely a genuine hammered metal finish, it is desirable to have the base material pigmented by grinding it with a pigment or dye designed to give an appropriate tint to the resulting finish. It is essential that a metallic bronze flake, preferably aluminum bronze, be incorporated in the finished product either by mixing or grinding. However, one may use copper, brass, bronze, gold or any other decorative flake metallic powder, although aluminum powder produces the best results because it tends to float or leaf readily and because its color produces a closer simulation of a hammered metal effect than do the other powders enumerated.

The metal powders or pastes used are coated with a fatty acid or soap and may be of the form commercially available. The quantity of metal powder per gallon of finished composition depends upon the particular metal powder or paste employed and also may be varied to produce different effects. It has been found that from  $\frac{1}{4}$  of 1% to 40% by weight of metal powder may be used for various effects, but the most practical and preferred range of metal powder is from approximately 1% to 5%.

The amount of granular pigment also varies greatly with the hiding power of the particular pigment employed and with the effect desired. Good results have been obtained from  $\frac{1}{4}$  of 1% to 30%, with the most satisfactory results and preferred range from 2% to 15% of pigment.

In the manufacture of the composition, it is relatively unimportant whether the pigmented enamel is added to the metallic flake or vice versa. The finished product is held in this state until required for application, at which time solvent is added to reduce the material within the range of good spraying consistency and the material sprayed, as described in the foregoing.

The spatter coat of thinner is then applied, the action of the droplets producing the hammered effect. Best results are obtained with a spray gun fitted with a spatter cap, although any type of equipment so adjusted or regulated as to spray in the form of droplets, rather than by a fine mist, will produce entirely satisfactory results. The thinner referred to above is composed of two or more miscible solvents, having relatively rapid rates of evaporation. The function of the thinner is to serve as a medium of movement in which the metallic particles concentrate towards the center and float towards the surface of each individual droplet, due to the violent and rapid ebullition of the volatile solvent. As a preferred thinner, I use a mixture consisting of equal parts by volume of denatured alcohol, methyl ethyl ketone and V. M. & P. naphtha. It is evident that a thinner, consisting of variations in the above combination or the solvents embracing slowly volatile or highly volatile solvents, or a single solvent, may be used, if desired.

As an example of a preferred coating composition spattered with thinner, the following pigmented resinous base material has been successfully applied:

*Example I*

|                            | Per cent |
|----------------------------|----------|
| Bone black                 | 3.18     |
| Iron oxide                 | 1.94     |
| Ferrite yellow             | .96      |
| Extra fine lining Al flake | 2.31     |
| Alkyd resin*               | 33.61    |
| Solvent                    | 58.00    |
|                            | 100.00   |

\* The alkyd resin of this example consisted of a blend of two synthetic resins, one being a linseed oil modified alkyd resin, and the other being a linseed and China-wood oil modified alkyd resin. These resins may be prepared by any method known in the art, but should preferably have a low acid number.

This material was applied on a smooth steel panel with a spray gun using 12-lb. fluid and 65-70 lb. air, holding the nozzle 12-15 inches from the surfaces. This enamel was immediately spattered with thinner using the combination consisting of ethyl alcohol, methyl ethyl ketone and V. M. & P. naphtha in equal parts by volume. The spatter coat was applied with a regular spatter gun using approximately 2-lb. fluid pressure and less than 15-lb. air pressure. The resulting film, after baking one hour at 225° F., showed a series of areas varying from  $\frac{1}{4}$  to  $\frac{1}{2}$  of an inch in diameter. The craters of the areas contained a high concentration of aluminum particles, tinted reddish gray, while the rim of the craters contained the base color of the pigment combination. This material can be modified, by incorporating suitable driers, to produce a satisfactory effect and hard film on air drying.

*Example II*

The following formula illustrates one embodiment of the invention in which nitrocellulose lacquer is used to produce an effect which closely simulates hammered metal and which may be applied to metal, wood or other surfaces:

|                                   | Per cent |
|-----------------------------------|----------|
| Nitrocellulose                    | 17.06    |
| Coconut oil modified alkyd resin* | 8.46     |
| Malic acid                        | .30      |
| Dibutyl phthalate                 | 3.63     |
| Extra fine lining aluminum paste  | 1.62     |
| Bone black                        | 2.37     |
| Titanium dioxide                  | 1.55     |
| Ramapo blue                       | .23      |
| Blown castor oil                  | 2.44     |
| Combined solvent and diluent      | 62.34    |
|                                   | 100.00   |

\*This resin is produced in any known manner and may contain approximately 34% coconut oil and 66% alkyd resin.

This lacquer was applied to the surface, as described in Example I, and the spatter coat of thinner sprayed immediately afterward. The resulting film, simulating a hammered appearance, was baked one hour at 180° F. to produce a hard film, although similar results can be obtained by air drying.

*Example III*

The following illustrates the invention where an oleoresinous type product is used which has produced a satisfactory hammered appearance. This finish is applied to a surface, as stated in Example I. The application of the spatter thinner, however, required a longer period of waiting to permit volatilization of the slower evaporating thinners with the best results being obtained at approximately fifteen minutes after the enamel was sprayed.

|                                                                            | Percent |
|----------------------------------------------------------------------------|---------|
| Bone black                                                                 | 17.00   |
| Extra fine lining aluminum paste (66.5% T. S.)                             | 1.87    |
| China-wood oil-limed rosin varnish (thirty gallon length—51% non-volatile) | 49.44   |
| Limed rosin (56% non-volatile)                                             | 10.33   |
| Lead-manganese drier                                                       | .59     |
| V. M. & P. naphtha                                                         | 5.09    |
| Mineral spirits                                                            | 15.68   |
|                                                                            | 100.00  |

50 The above paint, when applied on a steel surface, as previously described, and baked one hour at 225° F., produces a hard, dark gunmetal film, simulating a hammered finish.

55 While I have illustrated the invention with a resinous composition, a nitrocellulose lacquer, and an oil varnish vehicle, it is to be understood that the invention is not limited to the specific examples nor to the specific resin, cellulose derivative, or oil, since other resins which are capable of forming a durable film may be used. Likewise other cellulose derivatives such as cellulose acetate or cellulose ethers either alone or in combination with natural or synthetic resins are likewise suitable as far as producing the desired appearance is concerned. In place of China-wood oil, I may use linseed oil vehicles which may likewise contain resins.

60 While it is usually preferred to decorate wood, metal, or similar rigid bodies with a metallic finish, it is to be understood that the invention is not limited to these materials since paper, fabric of all kinds, and even other materials may be treated provided the surface is supported until the finish is sufficiently dry to prevent running or sticking when rolled.

It is apparent that many widely different embodiments of this invention may be made without departing from the spirit and scope thereof and therefore it is not intended to be limited except as indicated in the appended claims.

I claim:

1. The process of producing a simulated hammered metal finish which comprises applying to a rigid base a substantial film of a composition containing a film-forming agent, at least one volatile solvent, 2-15% granular pigment, and from 1-5% of a flake metallic powder, allowing the film to partially set by evaporation of the

solvent, immediately thereafter spattering thereon a composition consisting of highly volatile solvents for the film-forming agent, substantially in the form of coarse droplets under a fluid pressure of about 2 lbs. and an air pressure of less than 15 lbs. per sq. in. whereby the spattered solvent dissolves the film-forming agent and thereby forms apparent metallic craters, and drying the same to a hard finish.

2. The process of claim 1 in which the said solvent consists essentially of alcohol, methyl ethyl ketone, and naphtha.

GERALD E. ARMENTROUT.